

Nov. 3, 1942.

L. T. WELSHANS

2,301,101

106  
87

HOT TOP

Filed Sept. 26, 1940

Fig. 4



Fig. 1



Fig. 2



Fig. 3



Fig. 5

Inventor  
Lewis T. WelshansDodge *Att. J. J. J.*

By

Attorneys

XR

Al

## UNITED STATES PATENT OFFICE

2,301,101

## HOT TOP

Lewis T. Welshans, Charles Town, W. Va., assignor to The Standard Lime and Stone Company, Baltimore, Md., a corporation of Maryland

Application September 26, 1940, Serial No. 358,558

5 Claims. (Cl. 22—147)

This invention relates to hot tops used in conjunction with ingot molds to form a heat insulating extension at the top of the mold, which serves to retain a bath of molten metal at the top of the mold during the freezing of the ingot. The effect is to prevent or minimize piping and the formation of other defects in the head of the ingot.

In a prior application owned by applicant's assignee, and identified as Serial No. 282,259, filed June 30, 1939, in the name of I. A. Nicholas, there is described a hot top which is a decided improvement over the fire clay hot tops and the fire brick lined metal hot tops commonly used in the art. The present invention is in the nature of an improvement on the Nicholas invention.

The improved hot top hereinafter disclosed has a number of advantages as compared to prior art hot tops. These are: lightness, which permits a saving in the labor of placing the hot top; ease of manufacture from inexpensive materials with direct production economies; markedly increased heat insulating characteristics; and the characteristics of partially disintegrating at temperatures of molten steel with the result that portions of the hot top adhering to the ingot may be readily removed. Perhaps the most important characteristic is the fact that the material which forms the major component of the hot top is not harmful to the mill scale produced during the rolling of the ingot. On the contrary, it is beneficial.

The fire clay hot tops heretofore universally used are extremely difficult to remove when portions of them adhere to the ingot. This entails substantial labor costs in removal and when, as is often the case, the removal is not complete, the adhering fire clay is harmful to the ingot and even more harmful to the mill scale produced during rolling. Since mill scale is a commercial by-product of substantial value it is important that it not be contaminated.

According to the present invention the lightness of the hot top is increased by imparting a highly porous characteristic to the hot top or to the component slabs of which it may be composed. The material of which the hot top is composed comprises at least one basic carbonate such as magnesium or calcium carbonate, either artificially prepared or as they occur in nature. Dolomite may also be used. Sufficient hydraulic cement such as Portland cement is used as a binder, and with this Portland cement is used a gas generating substance such as pow-

dered aluminum which will generate gas in the presence of water by reaction with the alkaline constituents of the mix. Generally stated, the hydraulic cement is used only in sufficient quantity to produce the necessary binding action and is selected with reference to its setting characteristics to assure the desired porous texture. The quantity of powdered aluminum or its equivalent is determined on the basis of attainment of the desired porous texture. The texture is also affected by the setting time of the cement and the two must be suitably coordinated for best results.

When molten steel comes into contact with a hot top of this type, the carbonate will partially decompose leaving a powder of magnesium oxide or calcium oxide both of which have excellent insulating properties. The effect is to improve the heat insulating characteristic of the hot top during its use. Upon stripping, very little of the material of the hot top adheres to the ingot, and such as does adhere can readily be dislodged by poking with a rod. Any residue not dislodged readily falls off in the blooming mill rolls, and is not harmful to the mill scale. Mill scale is used in bain furnace and open hearth operations where its purity is an important factor. However, the residue from the improved hot top improves the smelting properties and, therefore, its presence is not objectionable whereas the presence of even small amounts of fire clay is most seriously objectionable.

The above being the general principle of the invention, the preferred mode of carrying it out will now be described in connection with the accompanying drawing in which:

Figure 1 is a perspective view of the hot top made up of four identical slabs cast from the material in question and connected by twisting together certain protruding reinforcing wires which are cast in the slabs;

Fig. 2 is a plan view of the hot top in position on the top of an ingot mold;

Fig. 3 is a vertical axial section of the upper portion of the mold with the hot top in place;

Fig. 4 is a face view of one of the slabs indicating the location of one form of reinforcement; and

Fig. 5 is a section through one of the slabs in the mold showing how the reinforcing material is placed and may be positioned during the slab casting operation.

The first step is to prepare the mix from which the slabs or hot tops are to be cast. Although a sectional hot top made up of slabs is shown and is

preferred, certain advantages of the invention can be had with hot tops cast in one piece as heretofore proposed.

A typical example using limestone as an ingredient will now be given: Limestone as it occurs in nature is pulverized and screened to a size under 8 mesh and over 60 mesh. To the pulverized limestone is added Portland cement in approximately equal quantity by weight. To these two ingredients is added 0.2% by weight of powdered aluminum. To the three ingredients above described an amount of water is added equal to about one-fourth of their combined weight. The ingredients are mixed in an ordinary concrete mixer. The resulting slurry is rather thin and can readily be poured into forms or molds to harden.

The powdered aluminum reacts with the water and the alkaline constituents of the mix to liberate gas which is trapped in the mix and causes puffing or swelling, resulting finally in a light weight porous slab. The swelling action ordinarily commences within fifteen minutes and the slabs will have set sufficiently within a few hours to permit their removal from the forms. After removal, they are allowed to cure, three days being considered the minimum curing period. The slabs are then dried until their water content is reduced to 1% or less. This can be conveniently accomplished by treating them in a drier at approximately 600° F. for twenty-four hours.

The resulting slabs are markedly porous and of sufficient strength to withstand shipping and handling. If stored, they should be kept dry and in a dry atmosphere, for they have a tendency to absorb moisture from the atmosphere. Excessive moisture in the slabs is objectionable during use because it causes the metal to boil.

Some reinforcement is desirable and I prefer to use a steel wire mesh fabric. A hexagonal mesh wire fabric of conventional weave is satisfactory. For slab-connection purposes I also use reinforcing wire strands which can be sustained by the wire mesh during the casting operation, which will now be explained in some detail, simply to disclose one commercially practicable procedure.

In Fig. 5 a portion of an open top mold is indicated at 6. Before the casting operation a sheet of reinforcing material such as hexagonal wire mesh fabric, indicated generally by the numeral 7, is placed in the mold and may be sustained by bending down strands of the mesh at the edge as indicated at 8. Strands of somewhat heavier wire indicated at 9 may be interlaced in the mesh with their end portions 11 bent outward so that they will protrude from the slab as indicated more clearly in Fig. 4.

The slurry or mix above described is poured into the mold, the quantity being such that after the swell takes place, the mold will be filled approximately to the level 12 (Fig. 5). The overhanging end 13 of the mold which produces the rounded end or fillet at one end of the slab may be made removable to facilitate removal of the slab from the mold after it has set. The resulting slabs can all be identical in size. Such slabs are generally indicated by the numeral 14 in Figs. 1 to 4.

For use with conventional ingot molds, two sizes of slab will suffice, one about 22½" by 15", and the other about 16½" by 15", the thickness being of the order of 2", though thinner slabs can be used. Four slabs of the larger size and of the 2" thickness stated, have a weight of about

100 pounds as compared with the weight of 200 pounds, or more, characteristic of the commercial hot tops of the prior art. The use of four slabs which are assembled to form the hot top reduces the storage space to about one fifth of that required where the hot tops are cast in one piece.

To produce the hot top, four slabs 14 are assembled as in Fig. 1, and the wires 11 are twisted together as indicated at 15 and thus connect the four slabs into a substantially unitary hot top. The hot top so formed is then inserted in the top of the ingot mold generally indicated at 16 in Figs. 2 and 3. The twisted wires 15 of the lower set engage the upper end of the ingot mold 16 and serve to sustain the hot top in position.

It has been stated that the material of which the slabs are composed tends to disintegrate at the temperature of molten steel. It should be explained that this disintegration is partial, and not attended by any danger, for the reason that a thin shell of steel instantly freezes within the hot top. Thus, contrary to prior belief, substantial mechanical strength of the hot top is by no means necessary. A crushing strength of 10 to 15 pounds per square inch obtainable with the porous slabs of the present invention is adequate despite the fact that the burned clay hot tops heretofore used had crushing strengths in some instances as high as 1500 pounds per square inch.

The insulating properties of the slabs are attributable to their porous or cellular texture and also to the inherent insulating properties of the pulverized ingredient which is used with the hydraulic cement. The preferred pulverized insulating ingredients are calcium carbonate, magnesium carbonate, or mixtures of calcium and magnesium carbonates in various proportions usually determined by the available supply. These carbonates are highly efficient thermal insulators. Their composition is such that they are not detrimental to mill scale and consequently they are preferred. It is, however, within the broad contemplation of the invention to use any other pulverized insulating material which will not react with the metal being cast or whose reaction therewith is tolerable. The described carbonates are believed to be the best available material.

The porosity and cellular texture may be produced in any known way, but the addition of the small percentage of aluminum is convenient and satisfactory. On the whole, aluminum is believed to be the best available substance because it can be readily obtained at a moderate price, has no objectionable reaction with the steel and does not begin to develop gas too soon or too suddenly. As a practical matter, it is desirable that the evolution of gas commence some minutes after the water has been added to the mixture, thus affording ample time for mixing and pouring. The time of evolution of the gas is also important with reference to the setting time of the cement for evolution should commence before setting starts and should be so timed as to secure the desired degree of porosity with the minimum reaction material. As a rule, use of one of the well known quick setting hydraulic cements is considered preferable.

A satisfactory slab can be produced by the use of the proportions outlined, but it must be understood that they are illustrative and not limiting. The effort is to use as little cement as is required for the binding effect and as little gas generating reagent as is necessary for the

desired degree of porosity. This permits avail-  
ing to the maximum degree of the desired chem-  
ical and heat insulating properties of the car-  
bonates.

It should be fully appreciated that the im-  
portant function of a hot top is to maintain as  
long as possible the molten condition at the top  
of the ingot mold and to avoid any harmful reac-  
tion with the molten metal. Consequently, the  
porous cellular structure, because of its markedly  
superior insulating qualities, represents a decided  
advance in the hot top art.

In its broadest aspects the invention contem-  
pates the use of the porous material in hot tops  
of any form, and in its more specific aspects  
involves its use with the suggested slab construc-  
tion and with the reinforcing and connecting  
stays as set forth. As has been suggested, con-  
siderable latitude in choice of materials and  
modification of proportions and time of drying  
are permissible.

What is claimed is:

1. In combination with an ingot mold, a cellu-  
lar insulating hot top supported by and forming  
a continuation of the top of said mold, said hot  
top comprising the reaction product of a slurry  
of a pulverized basic carbonate, a hydraulic ce-  
ment, and a powdered metal which in the pres-  
ence of water will react with alkaline ingredients  
of the slurry to generate porosity inducing gas,  
said hot top having the property of disintegrating  
to powder form when subjected to the heat of the  
molten metal poured into the mold.

2. In combination with an ingot mold, a cellu-  
lar insulating hot top supported by and form-

ing a continuation of the top of said mold, said  
hot top comprising a porous cellular mass of con-  
crete in which the aggregate is pulverized lime-  
stone bound by hydraulic cement, the concrete  
containing voids formed by gas bubbles evolved  
during the setting of the cement and serving to  
increase the heat insulating properties of the  
mass.

5 3. In combination with an ingot mold, a cellu-  
lar insulating hot top supported by and forming  
a continuation of the top of said mold, said hot  
top comprising a cellular mass consisting essen-  
tially of basic carbonate and hydraulic cement  
in substantially equal proportions, and having  
10 the property of disintegrating to powder form  
when subjected to the heat of the molten metal  
poured into the mold.

15 4. In combination with an ingot mold, a porous  
insulating hot top supported by the mold and  
forming a continuation of the mold top, said  
hot top being made up of separate slabs of cellu-  
lar concrete comprising a fine aggregate in the  
form of a basic carbonate and a bond in the form  
20 of hydraulic cement.

25 5. In combination with an ingot mold, a porous  
insulating hot top supported by the mold and  
forming a continuation of the mold top, said  
hot top being made up of assembled slabs each  
comprising a cellular mass of pulverized basic  
30 carbonate and hydraulic cement and having the  
property of disintegrating to powder form when  
subjected to the heat of the molten metal poured  
into the mold.

LEWIS T. WELSHANS.